

March 30, 1926.

1,578,609

W. H. MASON

# PROCESS AND APPARATUS FOR DISINTEGRATION OF WOOD AND THE LIKE

Filed Sept. 24, 1924



Patented Mar. 30, 1926.

1,578,609

# UNITED STATES PATENT OFFICE.

WILLIAM H. MASON, OF LAUREL, MISSISSIPPI.

## PROCESS AND APPARATUS FOR DISINTEGRATION OF WOOD AND THE LIKE.

Application filed September 24, 1924. Serial No. 739,748.

*To all whom it may concern:*

Be it known that I, WILLIAM H. MASON, a citizen of the United States, and a resident of Laurel, county of Jones, State of Mississippi, have invented a new and useful Improvement in Processes and Apparatus for Disintegration of Wood and the like, of which the following is a specification.

My invention relates to a process and apparatus for disintegration of ligno-cellulose materials, such as wood, for example. By application of my improved process, the disintegration of ligno-cellulose material, such as porous wood, for example, is so completely effected that it can be immediately subjected, without intermediate treatment, to the action of the ordinary beating and refining apparatus, such as used in paper mills in the manufacture of paper, and, after subjection to such apparatus, is available for manufacture of paper, board pulp, and the like.

According to the present invention the wood (which expression is used as a convenient designation for ligno-cellulose material generally) is preferably hogged or chipped into comparatively small pieces and is placed in a closed high pressure chamber, wherein it is subjected to a gaseous pressure as of steam, compressed air or the like, of at least 275# to the square inch, and preferably the pressure ranges from about 400 to 600# to the square inch. Where pressures over 275# and under 400# per square inch are made use of with wood not readily disintegrated, it is preferably subjected to successive disintegration steps to secure thorough disintegration, and this may be done when higher pressures are used, if desired. I have found that where the wood is discharged at pressures under 275# per sq. in. nothing more than a partial shredding is accomplished, and the material is not in condition for feeding directly to apparatus, such as paper mill beaters, for example. Steam is preferably used at least at the beginning of the operation since the softening action of steam on the wood is beneficial in securing a desirably high state of disintegration.

After the pressure has been maintained for a sufficient time to permit the gases under pressure to penetrate the wood and establish a substantial balance between internal and external pressure and temperature within and around the wood and to heat

the moisture within the wood to a temperature which will cause it to turn to steam upon release of pressure, an outlet valve of comparatively small dimension, as compared to the cross-section dimension of the main chamber, is opened. The pressure within the chamber causes the wood to be forcibly and progressively driven out through the valve opening, which may be and preferably is somewhat smaller in at least one dimension than the largest dimension of the pieces of wood introduced into the chamber. More or less compression of the wood as it passes the outlet appears to be useful in obtaining the best results in disintegration. During this progressive discharge the steam pressure or other source of pressure is preferably kept turned on and the pressure within the chamber maintained as far as possible, though there may be some reduction in pressure toward the end of the progressive discharge. In this way the last pieces discharged are disintegrated to substantially the same extent as those earlier discharged.

The pieces of wood as they progressively emerge are disrupted and disintegrated by the excess of internal pressure over external pressure, which last may be substantially atmospheric pressure, and with use of pressures as stated above the disintegration is so complete that the material can be subjected immediately, without intermediate treatment of any kind, to apparatus such as paper mill beaters, and when it comes from the beater or equivalent apparatus it is a pulp and is available for the manufacture of paper, pulp board, and the like.

In the accompanying drawings I have shown apparatus for carrying out the process. Fig. 1 is a diagrammatical sectional view of the preferred form of apparatus. Fig. 2 is a cross-sectional view of a water injector device, which may be substituted for the separator and conveyor of Fig. 1, and Fig. 3 is a section of the outlet valve on line 3-3, of Fig. 1.

The gun 10 containing the chamber or cylinder 12 and preferably heat insulated, as shown at 14, is preferably arranged vertically with a top inlet opening 16 closed by the taper valve 18. The means for operating valve 18 may consist of a steam cylinder 20 and piston 22 with control valves 24 and 26.

The chips 28 of wood are shown as supplied from a hopper 30 with a gate valve

32 for charging the gun through inlet 16. These chips are preferably of substantially uniform size, such, for example, as is common practice in preparing chips for digestors in the manufacture of chemical pulp.

The high pressure steam pipe 34 preferably is valve connected to chamber 12, as by connection 36 and 38, shown as arranged at the top and bottom ends of the gun re-

10 spectively.

A valve as compressed air pipe 40 may be supplied for admission of air or other gas under pressure. A draw off cock 41 serves for withdrawal of water of condensation and is preferably located at the lowest point in chamber 12.

The constricted outlet 42 in the gun base 44 is preferably of slot like form and preferably of uniform width and tapered at 20 the sides gradually narrowing downwardly (outwardly), as shown at 46, Fig. 3. To secure best results the section of the outlet should be less than one-tenth of the section of the cylinder bore.

15 A balanced slide valve is preferably provided to control outlet slot 42. In the form shown, gun base 44 includes a transversely extending valve cylinder 48 having guides for a valve rod 50, on which are arranged 10 the balanced valve members 52, 54. The valve may be operated by steam piston 56 in cylinder 58 controlled by hand valves 60, 62. The valve piston 52, which is used to open and shut off the outlet, is preferably provided with grooves 64, 64, in which the fibered wood accumulates and forms a seal, or piston rings may be used, if desired. In the closed position of the valve (see dotted lines in Fig. 1) one of these 35 grooves comes on each side of the outlet slot 42, so that valve leakage is effectually prevented. Adjustable stops, such as lock nuts 66, 68, may be provided to limit the valve movement. The outlet when the valve 40 is opened (at or toward the full line position of Fig. 1) is between pistons 52, 54, so that a balance is secured and the valve remains in any position in which it may be placed.

45 The space 70 between slide valve pistons 52 and 54 is greatly enlarged compared to the outlet slot 42, permitting ample room for expansion and disintegration of the pieces of wood as they emerge from slot 55 42, and the conduit 72, through which the disintegrated wood material passes rapidly, due to the force exerted behind it, and the change of the released steam from pressure energy to velocity energy, is likewise 60 of greatly increased cross-section as compared with outlet slot 42.

Conduit 72 may lead to a centrifugal separator 74 of known form, in which the steam or other expanding gas is discharged upward at 76 and the disintegrated wood dis-

charged tangentially falls to the outlet chute 78 and may be carried away to a beater or the like, as by means of a conveyor 80. The separator wall is preferably roughened where contacted by the discharged material, 70 and the discharged material passing over this roughened surface at high speed is thereby still further disintegrated.

If desired, especially where steam under pressure is made use of in the gun, the 75 conduit 72 may extend into contact with an annular source of water supply 82 giving practically an injector action, and the forcible contact of the water with the disintegrated material results in it being still 80 further disintegrated and broken up. The disintegrated wood is discharged with the water into any convenient tank or apparatus indicated diagrammatically at 84. Separation between solids and gases is in this 85 case not required, the steam being condensed on contact with the injector water. If desired, the disintegrated wood may be discharged from the pressure chamber directly into a tank or body of water. In these 90 or other ways the energy of the material discharged at high velocity may be utilized to assist in obtaining a desirably high state of disintegration of the wood. In the case 95 of resinous wood the steam discharge, as 76, may be carried to a condenser and the oily content as of turpentine and pine oil recovered by condensation and gravity separation, or where the product is blown directly into water the volatile resinous materials, as turpentine pine oil and the like, 100 may be recovered from the water.

While I have shown but a single gun in order to disclose the principle of the invention, it will be apparent that a number of 105 guns may be arranged in a battery to obtain practically continuous operation, and same can be used for obtaining successive disintegrations when desired.

Where white products or products free 110 from substantial discoloration are desired, I preferably make use of small wood chips of substantially uniform size about as produced for use in chemical digestors and introduce steam at first, holding it at a temperature and for a period of time which 115 will not result in discoloration of the disintegrated wood and products made therefrom. For example, I may steam the chips with steam at about 300# pressure per square inch for a period of about say one-half minute to one minute. If then the steam pressure is run up to about 400 to 600# per square inch for a few seconds, say in the neighborhood of about five seconds, and the discharge valve opened immediately, the disintegrated product is substantially white with practically no discoloration, and is well adapted for paper and the like products. Steam produced in a separate boiler is es- 120 125 130

sential in order to secure products at all free from discoloration. If the pressure is obtained by application of external heat direct to the gun, for example, the time required to produce the necessary pressure is so great that such products as can be obtained are very much discolored and even blackened, at least in part.

Instead of using steam to supply the additional pressure to produce the required disintegration, same may be supplied by means of compressed air, which may be made use of at a relatively low temperature, being in this respect unlike steam in which high pressure is always accompanied by a corresponding high temperature.

The operation will be readily understood. Valve 18 is opened and the wood introduced. Valves 18, 40, 41 and 52 being closed, the steam is turned on. Within a very short time the pressure is balanced within and without the pieces of wood and after preferably drawing off any water of condensation by valve 41, the outlet valve 52 is opened and the wood pieces progressively forced out are disintegrated at the outlet, the sound of discharge resembling an extremely rapid fire machine gun. The pressure is preferably kept turned on during the progressive discharge, and it is known when the charge of wood has been completely forced out by the sound of outrush of steam, whereupon the steam is shut off. At the end of discharge the upper steam valve 38 alone may be open. The steam pressure may be applied in graduated steps, if desired, as first at a pressure of about 350# per square inch, followed by a few seconds of steam at a pressure of 400-600# per square inch, as described above in connection with making products free from discoloration. If compressed air is made use of, as for keeping the temperature down with use of high pressure, steam is first admitted at a relatively low pressure, say about 200# per square inch for a sufficient interval to obtain a balancing of pressures and temperatures internally of and around the pieces of wood, then the steam valves are closed and the air valve 40 opened for a sufficient interval to secure the necessary high internal pressure before opening up the discharge valve 52. With air there is not the necessity for quick discharge in securing undiscolored products that there is with steam, since with air high pressures are not necessarily accompanied by high temperatures. While the valve 52 is of such construction that it can be closed when but part of the gun contents have been discharged, preferably the valve is left open until substantially the complete charge has been discharged.

It will be observed that the use of a constricted outlet port and of a balanced slide

valve in connection therewith are of great advantage in securing a progressive discharge, and in distributing the expenditure of released pressure over a comparatively long interval of time. In this way it becomes possible to make use of a pressure sufficiently high to secure effective disintegration of the wood upon release, and no substantial difficulties are encountered in the way of securing the gun against recoil or in the way of controlling or maintaining the valve as would be encountered, for example, with large area valves operating to release the pressure substantially simultaneously throughout the chamber, and also, of course, the excessive noise of explosion produced by the opening of such large area valves is avoided.

The disintegration operation of the present invention can be carried on at a very substantial saving in power, it requiring only about one-fifth to one-fourth of the horsepower days per ton of pulp produced by the ordinary grinding operation, besides being adapted, as below stated, to resinous woods not available for pulp manufacture by grinding.

Application of the present invention to resinous wood is of especial importance. Thorough disintegration is secured with little or no tearing or breaking of the fibre, which may be of substantially the normal maximum length. My invention enables such wood as southern pine, for example, to be used for pulp in paper manufacture and the like, and the disintegration operation is not interfered with by the presence of resinous materials as in the case of grinding, which is practically inapplicable to such woods as southern pine because of the resins gumming up the grinding wheels.

Grinding also tends to the production of short or broken fibre pulp. Because of this long fibre pulp, as sulfite pulp, is customarily added to ground wood pulp. Long fibre pulp made in accordance with my invention may be used for paper manufacture, if desired, without the addition of long fibre sulphite pulp, which is customarily added to ground paper pulp to give it the necessary strength.

In fact, long fibre pulp made in accordance with my invention may advantageously be used in place of the expensive sulphite pulp to give added strength to ground paper pulp at a very decided saving over the expense of sulphite pulp customarily used for this purpose.

Furthermore, the resinous material remaining in the pulp made from resinous wood in accordance with my invention of clean resins substantially freed from volatile oils, which are carried off with the steam, imparts to products made therefrom, as paper, pulp-board, or the like, water-

proofness and inkproofness to an extent which renders unnecessary or at least substantially reduces the need for the customary sizing treatment.

5 1. I claim:

1. The process of disintegrating ligno-cellulose material, which consists in subjecting same in substantially its natural state except for mechanical subdivision in a closed 10 high pressure chamber to penetration by elastic fluid under high pressure, and progressively forcing said material out through a relatively constricted opening in said chamber.

15 2. The process of disintegrating ligno-cellulose material, which consists in subjecting same in substantially its natural state except for mechanical subdivision in a closed high pressure chamber to penetration 20 by an elastic fluid such as steam, compressed air or the like, under high pressure, and progressively forcing said material out through a relatively constricted opening in said chamber, while maintaining a high 25 pressure therein.

3. The process of disintegrating ligno-cellulose material, which consists in placing said material in substantially its natural state except for mechanical subdivision in a 30 vertically arranged pressure chamber, subjecting same to penetration by an elastic fluid, such as steam, compressed air or the like, under high pressure, and progressively forcing said material out of said chamber 35 through a narrow opening in the lower end thereof, whereby discharge is in the direction of gravity.

4. The process of disintegrating ligno-cellulose material, which consists in placing 40 said material in a vertically arranged pressure chamber, subjecting same to the action of an elastic fluid, such as steam, compressed air or the like, under high pressure, and progressively forcing said material out of 45 said chamber through a narrow opening in the lower end thereof, while maintaining a high pressure within said chamber.

5. The process of disintegrating ligno-cellulose material, which consists in introducing same in the form of small pieces into 50 a closed high pressure chamber, subjecting same to the action of an elastic fluid, such as steam, compressed air or the like, under a pressure of about 350-600# per square 55 inch, and progressively ejecting same through a narrow outlet in the chamber.

6. The process of disintegrating ligno-cellulose material, which consists in introducing same in the form of small pieces 60 into a closed high pressure chamber, subjecting same to the action of an elastic fluid, such as steam, compressed air or the like, under a pressure of about 350-600# per square inch, and progressively ejecting same 65 through a narrow outlet in the chamber,

while maintaining a high pressure within said chamber.

7. The process of disintegrating ligno-cellulose material, which consists in placing said material in a closed high pressure 70 chamber, subjecting same to the action of steam under high pressure, progressively forcing said material out of said chamber through a narrow opening in the chamber wall while maintaining a high pressure 75 within said chamber, and injecting water into the stream of outgoing disintegrated material and steam, whereby the steam is condensed and the material more highly 80 disintegrated.

8. Apparatus for the disintegration of ligno-cellulose material comprising a high pressure cylinder, a valved inlet for charging said cylinder, means for the introduction of elastic fluid, such as compressed air, steam or the like, under high pressure, into said cylinder, a narrow outlet provided in the base of said cylinder, and a balanced slide valve for controlling the discharge of the material through said outlet.

9. Apparatus for the disintegration of ligno-cellulose material comprising a high pressure cylinder, a valved inlet for charging said cylinder, connections for introducing elastic fluid, such as compressed air, steam or the like, under high pressure, into said cylinder, a narrow outlet of gradually diminishing section provided in the base of said cylinder, and a steam operated balanced slide valve for controlling the discharge of the material through said outlet.

10. Apparatus for the disintegration of ligno-cellulose material comprising a high pressure cylinder, a valved inlet for charging said cylinder, connections for introducing elastic fluid under high pressure into said cylinder, a valve chamber adjacent to the base of said cylinder and extending transversely thereof, a narrow outlet of gradually diminishing section provided in the base of said cylinder and communicating with the valve chamber, and a balanced piston valve within said valve chamber for controlling the discharge of material from the cylinder through the narrow outlet.

11. Apparatus for the disintegration of ligno-cellulose material comprising a high pressure cylinder, a valved inlet for charging said cylinder, connections for introducing elastic fluid under high pressure into said cylinder, a valve chamber adjacent to the base of said cylinder and extending transversely thereof, a narrow outlet of gradually diminishing section provided in the base of said cylinder and communicating with the valve chamber, and a balanced piston valve within said valve chamber for controlling the discharge of material from the cylinder through the narrow outlet, said piston valve having annular grooves therein

12. Apparatus for the disintegration of ligno-cellulose material comprising a high pressure cylinder, a valved inlet with an outwardly closing valve for charging said cylinder, connections for introducing elastic fluid under high pressure into said cylinder, a valve chamber adjacent to the base of said cylinder and extending transversely thereof, a narrow outlet of gradually diminishing section provided in the base of said cylinder and communicating with the valve chamber, a balanced slide valve within said valve chamber for controlling the discharge of material from the cylinder through the narrow outlet, a steam cylinder and piston adjacent to the valve chamber and in alignment therewith, and a rod interconnecting the slide valve and steam cylinder piston, whereby the slide valve is actuated by movement of the piston within the steam cylinder. 10
13. Apparatus for the disintegration of ligno-cellulose material comprising a high pressure cylinder, a valved inlet for charging said cylinder, connections for introducing elastic fluid under high pressure into said cylinder, a valve chamber adjacent to the base of said cylinder and extending transversely thereof, a narrow outlet provided in the base of said cylinder and communicating with the valve chamber, a shaft in said valve chamber, two separated pistons within the valve chamber on said shaft, one of which is adapted to be moved in front of and away from said narrow outlet to control the discharge of material from the high pressure cylinder, and the other adapted to balance the pressure against the first named piston. 20
14. Apparatus for the disintegration of ligno-cellulose material comprising a high pressure cylinder, a valved inlet for charging said cylinder, connections for introducing elastic fluid under high pressure into said cylinder, a valve chamber adjacent to the base of said cylinder and extending transversely thereof, a narrow outlet of gradually diminishing section provided in the base of said cylinder and communicating with the valve chamber, a shaft extending axially through the valve chamber, and a balanced slide valve within said valve chamber on the shaft comprising two pistons substantially separated from one another, whereby a large expansion area is provided immediately upon the discharge of the material from the high pressure cylinder through the narrow outlet, and means for actuating the valve shaft to open and close the outlet valve. 30
15. A cylinder for pressure release disintegration of ligno-cellulose material having a relatively narrow outlet opening, and a balanced valve for said opening. 40
16. A cylinder for pressure release disintegration of ligno-cellulose material having a relatively narrow outlet opening, and a balanced piston slide valve for said opening. 50
17. The process of producing substantially undiscolored disintegrated wood, which consists in subdividing the wood into small pieces of substantially uniform size about as made use of in preparing chips for chemical reduction, applying steam thereto in a closed chamber at a pressure of about 275-350# per square inch for a relatively extended period, applying steam at a higher pressure of about 400-600# per square inch for a relatively short period, and then immediately discharging the contents of the chamber through a constricted orifice, whereby substantially undiscolored products are obtained. 60
18. The process of producing substantially undiscolored disintegrated wood, which consists in charging into a closed chamber small wood chips of substantially uniform size, subjecting same to a pressure of about 275-350# per square inch for a relatively extended period of say one-half minute to one minute, increasing the steam pressure to 400-600# per square inch for a relatively short period of a few seconds, and progressively discharging the contents of said chamber through a constricted orifice, whereby substantially undiscolored products are obtained. 70
19. The process of disintegrating wood, which comprises the steps of subjecting it in substantially natural state, except for mechanical subdivision, to penetration by steam under pressure of the order of 350# per square inch, and releasing the pressure. 80
20. The process of disintegrating wood, which comprises the steps of subjecting it, in substantially natural state except for mechanical subdivision, to penetration by steam under pressure of the order of 350# per square inch, then subjecting it to steam at a materially higher pressure (and temperature) for a relatively short time interval, and releasing the wood into a region where the pressure is not substantially in excess of atmospheric. 90
21. The process of disintegrating ligno-cellulose material, which consists in subjecting same in a closed high pressure chamber to penetration by an elastic fluid under pressure in excess of 275 pounds per square inch, and progressively discharging said material through a relatively constricted outlet from said chamber, whereby the expansion of the fluid is utilized for disintegrating said material. 100

In testimony whereof, I have signed my name hereto. 115

WILLIAM H. MASON. 125